

reference

## UNITED STATES PATENT OFFICE.

JOHANN FERLÀ, OF ST. GEORGE, NEW YORK, ASSIGNOR OF ONE-FOURTH TO CHARLES L. PARMELEE, OF ORANGE, NEW JERSEY.

## COMPOSITION-BOARD.

No. 909,173.

Specification of Letters Patent.

Patented Jan. 12, 1909.

Application filed September 8, 1906. Serial No. 333,805. Renewed April 1, 1908. Serial No. 424,538.

*To all whom it may concern:*

Be it known that I, JOHANN FERLÀ, a citizen of Switzerland, residing in St. George, county of Richmond, and State of New York, have invented new and useful Improvements in Composition-Boards, of which the following is a specification.

This invention relates to composition boards and has for its object the production 10 of a composition board which can be used as a substitute for wood, be worked with the same tools, be water-proof, fire-proof, acid-proof, and possess a high degree of electrical non-conductivity.

15 The invention also contemplates the production of a composition board which can be manufactured at low cost and which is characterized by great strength and durability.

The composition boards constructed according to the present invention are composed of Portland cement, hemp, asbestos, acetic acid, liquid glue, coloring matter in sufficient quantity.

In producing the composition board, the 25 asbestos and hemp are first cut and crushed into very small and fine pieces, almost to a powder, by means of special cutting machinery and a revolving crusher, after which these ingredients are mixed with cement and 30 coloring matter in the dry state. For this mixing a rotary machine or revolving kettle is preferably employed. The dry mixture of asbestos, hemp and coloring matter is then transferred to another mixer, where the nec-

essary quantities of acetic acid, liquid glue and water are added. The quantity of water added at this stage is sufficient to moisten the ingredients thoroughly and form a pasty mass. The mixture, which now contains all 35

the ingredients of the composition board, is transferred to a large tank provided with an agitator to prevent the solid material from settling or becoming hardened. From this tank the paste is transferred to a canal where 40 an excess of water is added to make the material flow freely. From this canal the paste flows into tanks of different size with outlets designed to permit the passage of the material in precisely the required quantity for 45 certain thicknesses.

The formation of the composition board from the highly fluid mixture in the tank is effected by allowing the material to flow on a moving or revolving metallic web to allow

the excess water to drain through the web, 55 which is preferably wire-cloth of suitable mesh; then the material is passed on to an endless strip of felt passing between adjustable rollers. The rollers gage the thickness of the sheet of composition board and the 60 felt serves to absorb a considerable portion of the water remaining in the mixture. Upon the felt the material becomes sufficiently hard to be handled, and as it passes from the felt it is cut by any suitable cutting mechanism 65 into sheets of the desired dimensions. These sheets of material are then carried to a powerful hydraulic press, where they are piled one upon another in such press as the capacity of the press allows. Each super- 70 posed layer is separated from the others by interposed pieces of sheet iron or steel, as otherwise the layers would all unite under pressure to form a single mass.

The present operation is carried on in a 75 vacuum, the pressure chamber being hermetically sealed at the beginning of the operation and being connected with two suction pumps, one at the top and the other at the bottom of the chamber. The former 80 pump removes air from the pressure chamber and from the material in the press, and the latter serves principally to remove the water from the material. In this manner sheets of composition board are produced which are 85 thoroughly homogeneous and entirely free from air-holes or pores.

Before the material is allowed to dry and immediately after leaving the hydraulic press, it may be pressed by means of dies into 90 any fancy design or shape or may be cut into ornamental patterns by means of suitable cutters. The material is then allowed to dry for seventy-two hours and is then dipped for a few seconds into water and allowed to dry 95 again. This final dipping into water and subsequent drying appears to have the effect of forming a superficial film upon the material, which is absolutely impervious to water.

100 The composition boards produced of the materials and according to the method above set forth is firm, solid, of great strength, fire-, water- and acid-proof, excellent insulating material and absolutely free from warping. 105 It may, however, be worked in precisely the same manner that wood is worked and without injury to ordinary wood-working tools.

Having thus described my invention, what I claim as new and desire to secure by Letters Patent is:

1. A composition of matter comprising in its composition Portland cement, mineral fiber, glue, and an acid solvent for glue.
2. A composition of matter comprising in its composition Portland cement, mineral fiber, acetic acid, and glue.

3. A composition of matter comprising in its composition Portland cement, asbestos, hemp, acetic acid, and liquid glue.

In testimony whereof, I have signed my name in the presence of two witnesses.

JOHANN FERLA.

Witnesses:

WM. BRADFORD,  
GILBERT GANNON.